

Patented Oct. 6, 1925.

## UNITED STATES PATENT OFFICE.

VICTOR S. ALLIEN, OF WILMINGTON, DELAWARE, ASSIGNOR TO DARCO CORPORATION, OF WILMINGTON, DELAWARE, A CORPORATION OF DELAWARE.

## RECOVERING OILS.

No Drawing.

Application filed January 19, 1922. Serial No. 530,454.

*To all whom it may concern:*

Be it known that I, VICTOR S. ALLIEN, a citizen of the United States, residing at Wilmington, in the county of New Castle 5 and State of Delaware, have invented certain new and useful Improvements in Recovering Oils, of which the following is a specification.

This invention relates to recovering oils; 10 and it comprises a method of utilizing used and dirty lubricating oil, such as "crank case oil," wherein such oil is submitted to a methodical purification, including a treatment with decolorizing carbon to remove 15 colloid matter including colloid carbon; all as more fully hereinafter set forth and as claimed.

The disposition of used and dirty lubricating oil is a difficult problem in many 20 cases, as in garages, machine shops, etc., and in such places it often becomes a nuisance. While derived from high grade oils and still containing much of the original material in chemically and physically unchanged state, 25 it is difficult to recover good lubricating oil from it, or indeed to do anything with it. In garages of any size there is frequently a large accumulation of what is known as "crank case oil," which may be taken as 30 typical of these waste oils. Crank case oil contains, in addition to the original lubricating oil, a greater or less proportion of more volatile oils of the nature of gasoline and kerosene; these volatile oils coming 35 partly from cracking of the lubricating oil by heat and partly by absorption from the explosive charge of the engine. It also contains carbon, finely divided metal and other solid matters. In part this solid material is 40 in coarse form but in part it is so fine as to be really of a colloid nature. This colloid, finely divided matter (carbon, etc.) is particularly hard to remove and is responsible for most of the difficulty in devising methods 45 of utilizing these waste oils.

I have found that a good grade of lubricating oil can be recovered from these waste materials by certain methodical treatments thereof; these treatments including one with 50 finely divided activated carbon of the nature of that which is now known on the market as "decolorizing carbon." A particularly good variety of this carbon is described and claimed in the Mumford Patent No. 1,286,187. 55 I find that on treating the oil at a proper

stage in the purification with decolorizing carbon of this nature, the colloid carbon of the oil is taken up and effectually removed by the decolorizing carbon, giving a bright, clear oil. Incidentally, the decolorizing 60 carbon often effects a considerable decolorization by removing dissolved coloring matters; but, for the present purposes, its power of removing colloided carbon and solids is more important. Where the matter in col- 65 loid suspension is substantially only carbon, as it frequently is, and particularly with crank case oil, or with any oil which has been settled or treated to remove coarse stuff, the result of the treatment of the oil with 70 the decolorizing carbon is to form a compound body of carbon of high pigmentary value. It may be used as a substitute for lampblack and the like. The colloid carbon of these used oils is of course in a state of 75 excessively fine division and of good pigmentary value. I regard the Mumford material as particularly advantageous for the present purposes since its carbon-gathering 80 power is much higher than that of other decolorizing carbons, so that not only is less of it required to do the necessary work but the pigmentary value of the compound carbon recovered is much greater owing to the high 85 proportion of colloid carbon therein.

In a specific embodiment of the present invention, treating crank case oil, the oil gathered up from the garages is allowed to settle for a time at the ordinary temperature to free it, as far as possible, of coarser 90 solid impurities. Usually it is allowed to settle about 24 hours. It is then separated from the mud, warmed and again settled. A temperature of about 130° F. and a settling period of about 12 hours are satisfactory. The separated impurities of both 95 these settling treatments may be filter-pressed to regain some of the oil and the solids of the press cake burned or otherwise disposed of. They may be burned to furnish lampblack. The material from the second or warm settling operation has considerable pigmentary value and it may be used for this purpose. After settling, the 100 warm oil may be passed through a suitable centrifugal machine adapted to remove further solids. The solids so separated are of better pigmentary value than those obtained in the second settling operation. The oil 105 is next heated in any suitable steam still to 110

remove gasoline and kerosene. Any still provided with means for introducing low pressure steam may be used for this purpose. Instead of stripping the oil of volatiles by steam it may be filmed out over heating surfaces in appropriate apparatus of well known types, with or without the use of vacuum, but steam distillation is ordinarily simpler and better. After passing in steam for a time, the lubricating oil becomes free of volatile oils and resumes its original high flash and fire tests. The volatile oils (gasoline and kerosene) recovered in steaming may be treated and utilized in any suitable manner, not here important. Finally it is best to pass the oil once more through a centrifugal to remove any solid matter separated in the heating operation.

In this procedure if decolorizing carbon is used at one or more points in the succession of steps just described the final product is a good and useful lubricating oil. The decolorizing carbon may, for example, be added to the oil after the warm settling and before the first treatment in a centrifugal. In so doing, the centrifugal removes the added decolorizing carbon as well as the colloid matter taken up by it, and the oil is more easily handled in the steam still. Or the decolorizing carbon may be added to the oil after the first treatment in a centrifugal and prior to distillation. In so doing, it goes into the still with the oil and is removed in the subsequent treatment in a centrifugal. Or it may be added after the distillation with steam and prior to the second treatment in a centrifugal. Added at any point in the succession of steps, it has the result of removing colloided matter as well as dissolved impurities and of facilitating the subsequent treatments.

Ordinarily, after all the treatments described, I give the oil a final treatment with fuller's earth. By using the decolorizing

carbon somewhere in the succession of steps prior to the use of fuller's earth, the amount of fuller's earth required is very little thereby making not only a saving in the amount of fuller's earth otherwise necessary to effect any substantial purification of the oil but in the amount of oil which must be lost in discarded earth. The use of fuller's earth alone with oils of this class in such a process as that just stated is very unsatisfactory; but where decolorizing carbon has been used in the manner described for removing colloid carbon during the purification operation, the use of fuller's earth is here as satisfactory as with other oils in the ordinary methods of treatment.

In the stated method of operating oil of uniform quality and light color is easily obtained.

The use of fuller's earth is not necessary in the present method, although it is often convenient. Decolorizing carbon used in the manner stated will give a satisfactory product without the use of fuller's earth.

Ordinarily, in the steam still, I raise the temperature of the oil to about 450 to 500° F. and continue the distillation until a residual oil of a flash point of about 420° is obtained.

What I claim is:—

In the treatment of crank case oil and the like to recover lubricating oil therefrom, the process which comprises settling said oil in a warm condition, removing further impurities by centrifugal action, steaming the oil to free it of volatile oils, removing solids by centrifugal action and finally treating with fuller's earth, an addition of decolorizing carbon being made to the oil prior to one of the centrifugal separations.

In testimony whereof, I have hereunto affixed my signature.

VICTOR S. ALLIEN.